# EUROPEAN PATENT SPECIFICATION

(11) **EP 0 873 393 B1**
(45) Date of publication and mention of the grant of the patent: **29.03.2000**
(21) Application number: 96937246.5
(22) Date of filing: 23.10.1996
(51) Int. Cl.: C11D 17/00, C11D 7/16, C11D 7/06, C11D 3/06

(54) **SOLID DETERGENT BLOCK**
FESTER REINIGUNGSMITTELBLOCK
BLOC DETERGENT SOLIDE

(30) Priority: 13.11.1995 EP 95203080
(43) Date of publication of application: 28.10.1998
(73) Proprietor: UNILEVER N.V., 3013 AL Rotterdam (NL); UNILEVER PLC, London EC4P 4BQ (GB)
(72) Inventor: VAN DEN BROM, Guido, Clemens, NL-3603 AN Maarssen (NL); CONNOTTE, Hendrik, Johannes, J., NL-3603 AN Maarssen (NL)
(74) Representative: Rosen Jacobson, Frans Lucas M.
(86) International application number: EP9604658
(87) International publication number: WO9718292

(56) References cited:
- EP-A- 0 297 273
- EP-A- 0 375 022
- WO-A-93/01266
- DE-C- 4 229 650

## Description

### Field of the invention

The present invention relates to a solid detergent block for obtaining an aqueous chemical solution having a substantially constant concentration. The invention also relates to a process for preparing such a block. Such detergent blocks are suitable for use in an industrial cleaning process, particularly a mechanical warewashing process, and generally comprise alkaline agents and detergency builders.

### Background of the invention

Industrial warewashing machines generally comprise a wash tank which contains the cleaning solution for the wash process. In this process, the soiled wash load is doused with the cleaning solution and subsequently with rinse water which falls into the wash tank. Each cycle, the cleaning power of the cleaning liquor is reduced, first because some is exhausted by the soil-removing process and, secondly, because it is diluted with rinse water. The cleaning solution is therefore recharged from time to time by adding fresh cleaning product from a dispenser system, which usually provides liquid product or a concentrated aqueous solution of a composition including solid chemicals.

A number of techniques are known for converting solid chemicals into a concentrated aqueous solution, dependent on the nature of the solid. For example, according to US patent 2,371,720 a solid powdered chemical can be dissolved by placing it on a sieve and spraying water on to said sieve from below.

Alternatively, the powdered material can be dissolved in a dispenser of the "water-in-reservoir" type. In this type of dispenser, the powdered material is submerged under water, which therefore becomes loaded or even saturated with the powder. When more water is added, the excess solution flows into an overflow pipe leading to the washing machine.

It is also possible to use solid detergent materials in the form of briquettes such as, for instance, described in US patents 2,382,163, 2,382,164 and 2,382, 165. Briquettes can be used with a "water-in-reservoir" type of dispenser.

A well-known type of solid detergent is the cast block form, whereby a solid detergent block having a weight of several kilograms is formed by pouring a concentrated aqueous slurry into a container, in which it solidifies upon cooling as a result of the hydration of the salts in the composition. Such cast solid blocks are, for example, described in European patent 3,769.

These solid blocks cast in containers require dispensing systems whereby water is sprayed onto the block while it is inside the container, thereby gradually dissolving the exposed surface to form a concentrated solution. Such a dispenser system is, for instance described in European patent application 244,153.

Solid detergent blocks have won a certain degree of popularity in the area of industrial warewashing because they constitute a non-dusty and therefore relatively safe product form for the often aggressive chemicals used. Furthermore, hydrated solid blocks are economical in use because they can be manufactured and transported as concentrated products. However, elevated temperatures are required in the manufacturing process of these hydrated solid detergent blocks and these temperatures have an adverse effect on the stability of heat-labile components of the blocks.

In EP-A-375,022, an alternative type of detergent block is disclosed, namely a block of compressed granular material. This block constitutes an even more concentrated product and enables the incorporation of heat-labile components such as bleach compounds.

However, we have found that the quality of these compressed detergent blocks often leaves to be desired when considerable levels of hygroscopic materals, such as caustic, are present therein.

We have now surprisingly found that optimal quality of compressed detergent blocks can be realised when detergent blocks having a composition according to the present invention are prepared. More in particular, we have found that rather specific compositions including a compressing aid and having controlled free water levels are essential for obtaining optimal quality of the detergent block. In the context of the present invention, a good quality block is defined as a block having a bulk density of 1200-2100 kg/m³, preferably 1700-2000 kg/m³, and showing neither cracks in the block (lamination) nor at the top or bottom surface of the block (capping).

### Definition of the invention

Accordingly, in a first aspect the present invention provides a solid detergent composition suitable for use in an industrial warewashing process and in the form of a block of compressed granular material, said block having a weight of 0.2-10 kg and comprising:
- 25 - 35%: by weight of an alkalimetal hydroxide selected from sodium- and potassium hydroxide;
- 40 - 55%: by weight of a phosphate builder;
- 1 - 3 %: by weight of a compressing aid selected from low foaming nonionic surfactants, metal soaps, paraffins, talcum powder, polyethylene glycol, sodium benzoate, mixtures of long chain ketones having more than 25 carbon atoms and fatty alcohols, and mixtures thereof; and
- up to 6%: by weight of free water.

Preferably, the detergent block according to the present invention has a weight of 1-5 kg.
In a second aspect, the present invention provides a process for manufacturing a solid detergent block of the invention, whereby a powder having a corresponding composition is compressed in a mould under a pressure of 3-30 kN/cm² to form a solid block.
A third aspect of the present invention is the use of a solid detergent block according to the invention in an industrial warewashing process.

### Detailed description of the invention

The solid detergent blocks of the invention generally contain detergent components usually found in detergent material suitable for use in a machine warewashing process. As shown above, these components comprise an alkalimetal hydroxide, a phosphate builder, and one or more types of compressing aid.

Owing to the relatively low alkalimetal hydroxide level of the detergent blocks of the invention, the moisture sensitivity is reduced during manufacturing of said blocks. This is of importance since it was found that the free water content of the detergent blocks must be below 6% by weight in order to obtain good quality blocks. A free water content above this level was found to result in lamination and capping phenomena, and or in considerable block expansion by which the lifetime and the block density are dramatically reduced. A high block density of at least 1700 kg/m³ is preferred since transport cost and amount of packaging material are generally reduced with blocks of higher density.

Control of the free water level during manufacture of the detergent blocks of the invention was found to be essential to obtain good quality blocks. Preferably, the free water level of the detergent blocks is below 4% by weight.
In the context of the present invention, free water level is defined as the weight loss observed when heating the granular material used for producing the block concerned, during 4 hours at a temperature of 130°C.

### Alkalimetal hydroxide

The type of alkalimetal hydroxide preferably used in the blocks of the invention, is sodium hydroxide.
In addition to alkalimetal hydroxide, the blocks of the invention may contain up to 20% by weight of other types of alkaline agent, preferably sodium- or potassium-metasilicate, or -carbonate.

### Phosphate builder

Generally, the detergent blocks of the invention contain 40-55% by weight of phosphate builder. This relatively high concentration range of phosphate builder, in combination with the relatively low level of alkalimetal hydroxide, makes the blocks extremely suitable for use with hard water.

The phosphate builder material present in the blocks of the invention is generally defined to be phosphate containing material which is capable of reducing the level of free calcium and magnesium ions in the wash liquor, and, preferably, provides the composition with other beneficial properties such as the generation of an alkaline pH and the suspension of soil removed from the substrate to be removed. Preferred phophate builders are pyrophosphate, orthophosphate and tripolyphosphate. Sodium tripolyphosphate is most preferred.

### Compressing aid

The compressing aid present in the blocks of the invention is selected from low foaming nonionic surfactants,such as C₈-C₂₀ alkoxylated fatty alcohols, metal soaps, paraffins, talcum powder, polyethylene glycol, sodium benzoace, mixtures of long chain ketones having more than 25 carbon atoms and fatty alcohols, and mixtures thereof.
This compressing aid is an essential ingredient of the detergent block of the invention since it is needed during the compaction process for obtaining strong blocks of good quality. However, only moderate levels of compressing aid, being in the range of 1-3% by weight, are required since levels above said range would result in weaker blocks.

Preferred compressing aids are mixtures of long chain ketones having more than 25 carbon atoms and fatty alcohols, since such mixtures are highly effective both as a lubricant during the manufacturing process of the block and as an anti-foaming agent when using the block in a machine warewashing process. These mixtures are preferably in the form of a dispersion of the long chain ketone in the liquid-form fatty alcohol which is preferably a branched tatty alcohol having 8 to 24 carbon atoms. Such compositions are commercially available, for instance from Henkel as Dehypon 2429™.

### Bleaching agent

The detergent block of the invention may also comprise a bleach component, encapsulated or not, in an amount of up to 20% by weight. Said bleach component may be a hypohalite bleach such as NaDCCA, or a peroxygen compound, i.e. a compound capable of yielding hydrogen peroxide in aqueous solution.
For environmental reasons, a peroxygen compound selected from alkali metal peroxides, organic peroxides, such as urea peroxide, and inorganic persalts such as the alkali metal perborates, percarbonates, perphosphates, persilicates and persulphates, is preferably used. Mixtures of two or more of such compounds may also be suitable.

Particularly preferred are sodium perborate tetrahydrate and, especially, sodium perborate monohydrate. Sodium perborate monohydrate is preferred because of its high active oxygen content. Sodium percarbonate may also be preferred for environmental reasons.
The peroxygen bleach compound is suitably present in the detergent block of the invention at a level of up to 20% by weight, preferably of from 5 to 10% by weight.
On the other hand, the hypohalite bleach, if present, may be suitably used in an amount of up to 5%, preferably 1-4% by weight, as active chlorine.

Organic peroxyacids may also be suitable as peroxygen bleaching agent. Such materials normally have the general formula: wherein R is an alkylene or substituted alkylene group containing from 1 to about 20 carbon atoms, optionally having an internal amide linkage; or a phenylene or substituted phenylene group; and Y is hydrogen, halogen, alkyl, aryl, an imido-aromatic or non-aromatic group, a C00H or group or a quaternary ammonium group.

Typical monoperoxy acids useful herein include, for example:
(i) peroxybenzoic acid and ring-substituted peroxybenzoic acids, e.g. peroxy-α-naphthoic acid;
(ii) aliphatic, substituted aliphatic and arylalkyl monoperoxyacids, e.g. peroxylauric acid, peroxystearic acid and N,N-phthaloylaminoperoxy caproic acid (PAP); and
(iii) 6-octylamino-6-oxo-peroxyhexanoic acid.

Typical diperoxyacids useful herein include, for example:
(iv) 1,12-diperoxydodecanedioic acid (DPDA);
(v) 1,9-diperoxyazelaic acid;
(vi) diperoxybrassilic acid; diperoxysebasic acid and diperoxyisophthalic acid;
(vii) 2-decyldiperoxybutane-1,4-diotic acid; and
(viii) 4,4'-sulphonylbisperoxybenzoic acid.

Also inorganic peroxyacid compounds are suitable, such as for example potassium monopersulphate (MPS).
If organic or inorganic peroxyacids are used as the peroxygen compound, the amount thereof will normally be within the range of about 2-10 % by weight, preferably from 4-8 % by weight.

All these peroxide compounds may be utilized alone or in conjunction with a peroxyacid bleach precursor and/or an organic bleach catalyst not containing a transition metal.

Peroxyacid bleach precursors are known and amply described in literature, such as in the British Patents 836988; 864,798; 907,356; 1,003,310 and 1,519,351; German Patent 3,337,921; EP-A-0185522; EP-A-0174132; EP-A-0120591; and US Patents 1,246,339; 3,332,882; 4,128,494; 4,412,934 and 4,675,393.

Another useful class of peroxyacid bleach precursors is that of the cationic i.e. quaternary ammonium substituted peroxyacid precursors as disclosed in US Patent 4,751,015 and 4,397,757, in EP-A0284292 and EP-A-331,229. Examples of peroxyacid bleach precursors of this class are:
2-(N,N,N-trimethyl ammonium) ethyl sodium-4-sulphonphenyl carbonate chloride (SPCC);
N-octyl,N,N-dimehyl-N₁₀-carbophenoxy decyl ammonium chloride (ODC);
3-(N,N,N-trimethyl ammonium) propyl sodium-4-sulphophenyl carboxylate; and
N,N,N-trimethyl ammonium toluyloxy benzene sulphonate.

A further special class of bleach precursors is formed by the cationic nitriles as disclosed in EP-A-303,520 and in European Patent Specification No.'s 458,396 and 464,880.

Any one of these peroxyacid bleach precursors can be used in the present invention, though some may be more preferred than others.

Of the above classes of bleach precursors, the preferred classes are the esters, including acyl phenol sulphonates and acyl alkyl phenol sulphonates; the acyl-amides; and the quaternary ammonium substituted peroxyacid precursors including the cationic nitriles.

Examples of said preferred peroxyacid bleach precursors or activators are sodium-4-benzoyloxy benzene sulphonate (SBOBS); N,N,N'N'-tetraacetyl ethylene diamine (TAED); sodium-1-methyl-2-benzoyloxy benzene-4-sulphonate; sodium-4-methyl-3-benzoloxy benzoate; SPCC; trimethyl ammonium toluyloxy-benzene sulphonate; sodium nonanoyloxybenzene sulphonate (SNOBS); sodium 3,5,5-trimethyl hexanoyloxybenzene sulphonate (STHOBS); and the substituted cationic nitriles.

The precursors may be used in an amount of up to 12 %, preferably from 2-10 % by weight, of the composition. Organic bleach catalyst most suitable for being utilized here are the so-called sulphonimides as disclosed in EP-A-0453,003 and EP-A-0446,982.

### Other ingredients

The detergent block of the invention preferably also comprises 0-10% by weight of a polycarboxylated polymer. Suitable polymers are for instance polyacrylates such as Norasol LMW45D™, ex Norsohaas.
However, a polycarboxylate polymer on a suitable carrier material, for instance a polyacrylate polymer on a carbonate and/or silicate carrier, such as Norasol WL2-Si™, ex NorscHaas, is more preferred. Reason is that the presence of this type of polymer on carrier in the detergent block, desirably at a level up to 25% by weight, results in a higher density and improved stability of the block.

The detergent block of the invention may further comprise suitable minor ingredients, such as bleach stabilizers, enzymes, etc.

### Process

During manufacture of the detergent block of the invention, it is preferred that all solid starting materials should be dry and (in the case of hydratable salts) in a low hydration state. For instance, anhydrous phosphate builder is preferably used as constituent of the detergent block.

According to the process of the invention, a suitable granular detergent powder corresponding to the desired chemical composition is formed and subsequently compressed in a mould under a pressure of 3-30 kN/cm². Preferably, all constituents of the detergent block are homogeneously distributed through the powder before compression of said powder is carried out.

This process can be carried out in any suitable press, preferably a hydraulic press containing two movable punches, for instance a LAEIS Hydraulische Doppeldruckpresse, TYP HPF 630 as manufactured by LAEIS, West Germany.

In order to obtain good quality blocks having a sufficiently low free water content, the relative humidity of the air that is contact with the powder to be compacted during the manufacturing process, is preferably kept below 35%, more preferably below 10% .
Preheating of the powder to be compacted or heating of the punches of the hydraulic press, generally results in reduced stickyness of said powder, which in turn leads to less wall friction of the detergent block in the mould, and, consequently, a reduced risk of damage when ejecting said block out of the mould. However, for safety reasons (in order to avoid any risk of self heating due to exothermic reactions) the powder temperature is preferably kept below 40°C, more preferably below 35°C.
Since the compaction is carried out at such moderate temperatures, considerable levels of heat sensitive components, such as bleach compounds, may be incorporated in the detergent block of the invention. This is regarded as an additional advantage of this manufacturing process. In order to minimize the risk of the occurrence of capping phenomena caused by air expansion, a deaeration step is preferably applied during the compaction process.
After manufacture, the detergent block of the invention is desirably packaged as soon as possible, owing to its hygroscopic nature.

### Use

Another aspect of the invention is the use of the solid detergent block of the invention in an industrial warewashing process. Owing to the relatively high phosphate builder content of the block of the invention, said block is very suitable for use with hard water.
In use, the detergent block may be placed inside a suitable dispenser, in which it is sprayed upon with water in order to obtain an aqueous solution of the solid detergent material. Depending on the nature of the solid detergent block or the invention, the water may also form a slurry or suspension of the chemical material contained therein.

The invention is further illustrated by the following nonlimiting Examples, in which parts and percentages are by weight unless otherwise stated.

In the Examples, the following abbreviations are used:

| | |
|---|---|
| Thermphos NW™ | sodium tripolyphophate, ex Hoechst; |
| Dehypon 2429™ | mixture of ketones in fatty alcohol, ex Henkel; |
| Norasol WL2-Si™ | 40% polyacrylate (mol wt 4500) on 30% sodium silicate (SiO₂:Na₂O=2) and 30% sodium carbonate, ex NorsoHaas |
| Caustic soda | sodium hydroxide micropearls, ex Solvay; |
| Na DCCA dihydrate | Na dichloroisocyanurate. dihydrate, ex FMC. |

### Example 1, Comparative Example A

Homogeneous powder-form mixtures having the following compositions were obtained by mixing the components in a Lodige-type mixer:

| Example no. | 1 (%) | A (%) |
|---|---|---|
| Thermphos NW™ | 50.0 | 32.0 |
| Dehypon 2429™ | 2.0 | 2.0 |
| Norasol WL2-Si™ | 12.5 | 12.5 |
| Caustic soda | 30.2 | 50.0 |
| Na DCCA dihydrate | 5.3 | 3.5 |

The free water content of the resulting powder was measured to be 3.4% by weight (for the mixture of Example 1) respectively 6.6% by weight (for the mixture of Example A).

In both cases, the resulting powder was compressed to 3 kg blocks in a mould under a pressure of 14 kN/cm² using a double punch press. During this compaction process, the temperature and relative humidity of the air that was in contact with the powder to be compacted, were respectively 28°C and 8%.

As a result blocks were obtained having following quality characteristics:

| Examples | 1 | A |
|---|---|---|
| block density (kg/m³) | 1780 | <1180 |
| appearance of block | strong | expanded |
| lamination | no | yes |
| capping | no | yes |
| cracks | no | yes |

It can be concluded that the block according to the invention has a significantly better quality than the block of the comparative Example having a free water content in excess of 6% by weight.

## Claims

1. Solid detergent composition suitable for use in an industrial warewashing process and in the form of a block of compressed granular material, said block being of the type having a weight of 0.2-10Kg and comprising an alkalimetal hydroxide, a phosphate builder and a compressing aid, the composition being characterised in that it includes:
25-35% by weight of the alkalimental hydroxide, wherein the alkalimetal hydroxide is selected from sodium - and potassium hydroxide;
40-55% by weight of the phosphate builder;
1-3% by weight of the compressing aid, wherein the compressing aid is selected from low foaming nonionic surfactants, metal soaps, paraffins, talcum powder, polyethylene glycol, sodium benzoate, mixtures of long chain ketones having more than 25 carbon atoms and fatty alcohols, and mixtures
thereof;
and up to 6% by weight of free water,
wherein free water is defined as the weight loss observed when heating the granular material used for producing the block during 4 hours at a temperature of 130°C.

2. Solid detergent composition according to claim 1, having a weight of 1-5 kg.

3. Solid detergent composition according to claim 1 or 2, wherein the phosphate builder is sodium tripolyphosphate.

4. Solid detergent composition according to any of claims 1-3, wherein the compressing aid comprises a mixture of a long chain ketone having more than 25 carbon atoms and a fatty alcohol.

5. Solid detergent composition according to any of claims 1-4, comprising up to 4% by weight of free water.

6. Solid detergent composition according to any of claims 1-5, additionally comprising up to 20% by weight of a bleaching agent.

7. Solid detergent composition according to claim 6, wherein said bleaching agent is selected from sodium perborate and sodium percarbonate.

8. Process for the manufacture of a solid detergent composition according to any of claims 1-7, whereby a powder having a corresponding composition is compressed in a mould under a pressure of 3-30 kN/cm² to form a solid block.

9. Process according to claim 8, whereby during said process the relative humidity of the air that is in contact with the powder to be compacted, is below 35%.

10. Process according to claim 8 or 9, whereby during said process the temperature of the powder to be compacted , is below 40°C.

11. Use of a solid detergent composition according to any of claims 1-7, in an industrial warewashing process.

## Patentansprüche

1. Feste Waschmittelzusammensetzung, geeignet zur Verwendung in einem industriellen Geschirrwaschverfahren und in Form eines Blocks aus verpreßtem, granulärem Material, wobei der Block von der Art ist, die ein Gewicht von 0,2-10 kg aufweist, und ein Alkalimetallhydroxid, einen Phosphatbuilder und eine Verpreßhilfe umfaßt, wobei die Zusammensetzung dadurch gekennzeichnet ist, daß sie einschließt:
25-35 Gewichtsprozent des Alkalimetallhydroxids, wobei das Alkalimetallhydroxid ausgewählt ist aus Natrium- und Kaliumhydroxid;
40-55 Gewichtsprozent des Phosphatbuilders;
1-3 Gewichtsprozent der Verpreßhilfe, wobei die Verpreßhilfe ausgewählt ist aus wenig schäumenden, nichtionischen Tensiden, Metallseifen, Paraffinen, Talkumpulver, Polyethylenglycol, Natriumbenzoat, Gemischen von langkettigen Ketonen mit mehr als 25 Kohlenstoffatomen und Fettalkoholen und Gemischen davon;
und bis zu 6 Gewichtsprozent freies Wasser,
wobei freies Wasser als der Gewichtsverlust definiert wird, der beobachtet wird, wenn das zur Herstellung des Blocks verwendete granuläre Material während 4 Stunden auf eine Temperatur von 130°C erhitzt wird.

2. Feste Waschmittelzusammensetzung nach Anspruch 1, mit einem Gewicht von 1-5 kg.

3. Feste Waschmittelzusammensetzung nach Anspruch 1 oder 2, wobei der Phosphatbuilder Natriumtripolyphosphat ist.

4. Feste Waschmittelzusammensetzung nach einem der Ansprüche 1 bis 3, wobei die Verpreßhilfe ein Gemisch eines langkettigen Ketons mit mehr als 25 Kohlenstoffatomen und einen Fettalkohol umfaßt.

5. Feste Waschmittelzusammensetzung nach einem der Ansprüche 1 bis 4, umfassend bis zu 4 Gewichtsprozent freies Wasser.

6. Feste Waschmittelzusammensetzung nach einem der Ansprüche 1 bis 5, zusätzlich umfassend bis zu 20 Gewichtsprozent eines Bleichmittels.

7. Feste Waschmittelzusammensetzung nach Anspruch 6, wobei das Bleichmittel aus Natriumperborat und Natriumpercarbonat ausgewählt ist.

8. Verfahren zur Herstellung einer festen Waschmittelzusammensetzung nach einem der Ansprüche 1-7, wodurch ein Pulver mit einer entsprechenden Zusammensetzung in einer Form zur Bildung eines festen Blocks unter einem Druck von 3-30 kN/cm² verpreßt wird.

9. Verfahren nach Anspruch 8, wobei während des Verfahrens die relative Luftfeuchtigkeit, die mit dem zu verdichtenden Pulver in Kontakt steht, unterhalb 35% ist.

10. Verfahren nach Anspruch 8 oder 9, wobei während des Verfahrens die Temperatur des zu verdichtenden Pulvers unterhalb 40°C ist.

11. Verwendung einer festen Waschmittelzusammensetzung nach einem der Ansprüche 1-7 in einem industriellen Geschirrwaschverfahren.

## Revendications

1. Composition détergente solide appropriée pour l'utilisation dans un procédé de lavage de la vaisselle industriel et sous la forme d'un bloc de matière granulaire comprimée, ledit bloc étant du type ayant un poids de 0,2 à 10 kg et comprenant un hydroxyde de métal alcalin, un adjuvant phosphate et un auxiliaire de compression, la composition étant caractérisée en ce qu'elle comporte :
25 à 35% en poids de l'hydroxyde de métal alcalin, l'hydroxyde de métal alcalin étant choisi parmi l'hydroxyde de sodium et de potassium,
40 à 55% en poids de l'adjuvant phosphate,
1 à 3% en poids de l'auxiliaire de compression, l'auxiliaire de compression étant choisi parmi les tensioactifs à faible moussage, les savons métalliques, les paraffines, la poudre de talc, le polyéthylèneglycol, le benzoate de sodium, les mélanges de cétones à chaîne longue ayant plus de 25 atomes de carbone et d'alcools gras et leurs mélanges,
et jusqu'à 6% en poids d'eau libre, l'eau libre étant définie comme la perte pondérale observée quand on chauffe la matière granulaire utilisée pour produire le bloc pendant 4 heures à une température de 130°C.

2. Composition détergente solide selon la revendication 1, ayant un poids de 1 à 5 kg.

3. Composition détergente solide selon la revendication 1 ou 2, dans laquelle l'adjuvant phosphate est le tripolyphosphate de sodium.

4. Composition détergente solide selon l'une quelconque des revendications 1 à 3, dans laquelle l'auxiliaire de compression comprend un mélange d'une cétone à chaîne longue ayant plus de 25 atomes de carbone et d'un alcool gras.

5. Composition détergente solide selon l'une quelconque des revendications 1 à 4, comprenant jusqu'à 4% en poids d'eau libre.

6. Composition détergente solide selon l'une quelconque des revendications 1 à 5, comprenant de plus jusqu'à 20% en poids d'un agent de blanchiment.

7. Composition détergente solide selon la revendication 6, dans laquelle ledit agent de blanchiment est choisi parmi le perborate de sodium et le percarbonate de sodium.

8. Procédé de fabrication d'une composition solide détergente selon l'une quelconque des revendications 1 à 7, dans lequel la poudre ayant une composition correspondante est comprimée dans un moule sous une pression de 3 à 30 kN/cm² pour former un bloc solide.

9. Procédé selon la revendication 8, dans lequel pendant ledit procédé, l'humidité relative de l'air en contact avec la poudre à comprimer est en dessous de 35%.

10. Procédé selon la revendication 8 ou 9, dans lequel pendant le procédé, la température de la poudre à comprimer est en dessous de 40°C.

11. Utilisation d'une composition solide détergente selon l'une quelconque des revendications 1 à 7, dans un procédé de lavage de la vaisselle industriel.
